

**1**

3,829,367

**ELECTROLYTIC POLISHING OF METALS**Samuel Raviv, 8 Deborah St.,  
Beer-Sheba, Israel

No Drawing. Continuation-in-part of abandoned application Ser. No. 101,437, Dec. 24, 1970. This application July 14, 1972, Ser. No. 271,933

Int. Cl. C23b 3/06

U.S. CL. 204—129.95

**10 Claims****ABSTRACT OF THE DISCLOSURE**

Electrolytic polishing of a metal body. In a first stage intergranular corrosion of the body is induced by electrolytic cathodic treatment in an acidic electrolyte containing a copper salt. In a second stage the polarity is reversed and the body is subjected to electrolytic anodic treatment. The electrolyte in the second stage may be the same as in the first stage or different.

The present invention is a continuation-in-part of my previous application Ser. No. 101,437 now abandoned.

The present invention concerns a method for the electrolytic polishing of aluminum and its alloys, copper and its alloys and stainless steels.

It is known to polish metal surfaces electrolytically by superficial anodic dissolution of the metal. In these processes, the metal body is immersed in a suitable electrolytic bath, connected to the positive terminal of a D.C. source and a second electrode is immersed in the same bath and is connected to the negative terminal of the same D.C. source, and direct electric current is allowed to flow in the circuit.

It has also been known to dissolve a metal body cathodically by immersing it in nitric acid, connecting it as cathode into an electrolytic circuit and allowing electric current to flow in the circuit until the desired degree of dissolution has occurred. This method is described in Israel Pat. No. 26,224 and corresponding foreign patents, such as French Pat. No. 1,549,365, British Pat. No. 1,129,750 and Belgian Pat. No. 704,472.

It has long been known that where a metal is completely immersed in an electrolyte, there occurs a deterioration of the metal which is referred to in the art as intercrystalline or intergranular corrosion (see, for example, "Théorie et Méthodes d'Essai de la Corrosion des Métaux" by G. V. Akimov, N. D. Thomashov (Dunod, Paris, 1957), p. 7, 290-296). This phenomenon is generally considered as a nuisance and nobody has so far considered controlling it and utilizing it for any constructive purpose.

In accordance with the invention it has now been surprisingly discovered that intergranular corrosion of metals can be enhanced electrolytically by a controlled cathodic treatment.

It has now further been discovered in accordance with the present invention that for an effective and controlled intergranular corrosion, the formation of hydrogen should be prevented and that this is best achieved by the incorporation of a copper salt in the electrolytic solution in which the cathodic treatment is effected.

Furthermore, in accordance with the invention, there has now been made yet another surprising observation that when, subsequent to the controlled intergranular corrosion, the metal is subjected to anodic treatment, the ridges and planar stretches between the fissures that resulted from the intergranular corrosion are dissolved whereby the metal surface is smoothed and becomes highly polished with a mirror-like lustre, of a quality far surpassing that obtained by conventional polishing methods. The above applies both when the body remains in the original electrolyte and when it is transferred to a different one.

**2**

When the said anodic treatment is followed by means of profilographic measurements of the metal surface, it is observed that the degree of polish of the surface increases up to a certain time, after which it remains practically unchanged. It is believed that this stage is reached when the ridges and planar stretches are completely levelled off to become flush with the bottom of the fissures that result in the first stage from intergranular corrosion. This is, however, merely a tentative explanation which should not be construed as limiting the invention in any way.

According to the invention there is thus provided a process for the electrolytic polishing of a body made of a metal selected from the group consisting of aluminum, aluminum alloys, copper, copper alloys and stainless steels, wherein in a first stage said body is subjected for at least one minute to an electrolytic cathodic treatment in an acidic electrolyte containing a copper salt in an amount not exceeding 10 g./l. thereby to cause intergranular corrosion to occur in the surface region of said body, and in a subsequent, second stage, said body is subjected to electrolytic anodic treatment for at least one minute thereby to impart to the body a desired degree of polish, the following conditions being maintained throughout said first and second stages:

25 Voltage \_\_\_\_\_ volts 5-150  
Current density on the body \_\_\_\_\_ amp./dm.<sup>2</sup> 1-150  
Electrolytic bath temperature \_\_\_\_\_ ° C 20-95

Preferably, the amount of copper salt incorporated in the electrolytic solution used for the cathodic treatment is within the range of 1-10 g./l. An example of a copper salt suitable for the purposes of the present invention is copper sulfate.

The acidic electrolytic solutions suitable for use in the method according to the invention are aqueous, but may also contain varying proportions of organic solvents, in particular lower aliphatic alcohols or polyalcohols.

The polish of the metal surface produced in accordance with the invention is of superior quality as can easily be established by the eye. The invention is thus useful in a variety of cases where high polished metal surfaces are required, e.g. in the production of metal light reflectors and mirrors, in the formation of highly polished areas on the surfaces of various metal appliances for ornamental purposes and the like.

A specific application that deserves special mentioning concerns high vacuum equipment. In such equipment the inner surfaces of all components must have a high polish in order to reduce as much as possible to gas adsorption thereon. The polish achieved by hitherto known techniques was not quite satisfactory in this respect. Against this, surfaces polished in accordance with the present invention have been found virtually not to adsorb any gas and, consequently, the techniques of the present invention can successfully be applied for polishing surfaces of high vacuum equipment.

If desired, it is possible in accordance with the invention to polish the surfaces of a metal body selectively. One way of achieving this is to immerse the body only 60 partly in the aqueous electrolytic solution at least during the second stage. In this way the finished body comprises two zones—a polished one and a non-polished one.

Another way of achieving selective polishing, applicable when non-polished and polished zones are mutually interspersed, is to cover the body selectively, at least during the second stage, by insulating material not affected by the electrolytic solution. In consequence only the non-covered portions of these surfaces are polished. After the completion of the polishing the insulating material is removed. The insulating material may, for example, be a varnish or a plastic material which is applied by spraying, spreading, brushing or the like and is at the end of an operation.

In some cases it may be desirable to connect the metal electrically prior to its immersion in the electrolyte in order to ensure in this way that from the outset the con-

1-3. The electrolytic solutions and the conditions used in the process are listed in Table 2. In all cases a highly polished surface was obtained.

TABLE 2

| Ex. No. | Composition of the electrolytic bath                                                                                                                                | Voltage in volts | Current density, amp/dm. <sup>2</sup> | T cathode, minutes | T anode, minutes | Temperature, °C. |
|---------|---------------------------------------------------------------------------------------------------------------------------------------------------------------------|------------------|---------------------------------------|--------------------|------------------|------------------|
| 4       | H <sub>3</sub> PO <sub>4</sub> , 85%; Propyl alcohol, 15%; CuSO <sub>4</sub> , 7 g./l.                                                                              | 15               | 30                                    | 3                  | 5                | 55               |
| 5       | H <sub>3</sub> PO <sub>4</sub> , 70%; butyl alcohol, 30%; CuSO <sub>4</sub> , 6 g./l.                                                                               | 15               | 30                                    | 3                  | 6                | 40               |
| 6       | H <sub>3</sub> PO <sub>4</sub> , 65%; glycerine, 35%; CuSO <sub>4</sub> , 5 g./l.                                                                                   | 20               | 40                                    | 4                  | 8                | 90               |
| 7       | H <sub>3</sub> PO <sub>4</sub> , 60% plus H <sub>2</sub> SO <sub>4</sub> , 40% to which mixture is added: CrO <sub>3</sub> , 7.5 g./l.; CuSO <sub>4</sub> , 4 g./l. | 15               | 60                                    | 1                  | 5                | 80               |

trolled electrolytic phenomena prevail over any possible purely chemical attack which might otherwise prevail at the start.

The mechanical means by which the body is connected to a D.C. source and retained suspended in the electrolytic bath are conventional and do not form part of the invention. They need consequently not be described.

The following Examples illustrate the use of the method according to the invention for the polishing of a number of metals, it being understood that the invention is not

The same solutions may also be applied for polishing copper, aluminum and their alloys.

15

## EXAMPLES 8-11

Bodies made of copper, copper-zinc alloys and copper-zinc-nickel alloys, were submitted to a procedure analogous to that described for Examples 1-3. The electrolytic solutions and the conditions used in the process are listed in Table 3. In all cases a highly polished surface was obtained.

TABLE 3

| Ex. No. | Composition of the electrolytic bath                                                                                          | Voltage in volts | Current density, amp/dm. <sup>2</sup> | T cathode, minutes | T anode, minutes | Temperature, °C |
|---------|-------------------------------------------------------------------------------------------------------------------------------|------------------|---------------------------------------|--------------------|------------------|-----------------|
| 8       | H <sub>3</sub> PO <sub>4</sub> , 35%; H <sub>2</sub> O, 75%; CuSO <sub>4</sub> , 5 g./l.                                      | 12               | 20                                    | 5                  | 5                | 20              |
| 9       | H <sub>3</sub> PO <sub>4</sub> , 60%; isopropyl alcohol, 40%; CuSO <sub>4</sub> , 7 g./l.                                     | 12               | 30                                    | 2                  | 5                | 30              |
| 10      | H <sub>3</sub> PO <sub>4</sub> , 75%; sec.butyl alcohol, 25%; CuSO <sub>4</sub> , 9 g./l.                                     | 15               | 30                                    | 2                  | 8                | 40              |
| 11      | H <sub>3</sub> PO <sub>4</sub> , 40%; glycerine, 20%; butyl alcohol, 20%; H <sub>2</sub> O, 20%; CuSO <sub>4</sub> , 10 g./l. | 15               | 25                                    | 2                  | 8                | 40              |

limited to the conditions specified therein. In all the Examples the metal bodies that were polished were first degreased, e.g. chemically by cleansing with an organic solvent, or electrochemically, both as known per se, and then rinsed with water, before being subjected to the polishing treatment according to the invention. After completion of the second stage of the treatment the bodies were rinsed with water and dried.

## EXAMPLES 1-3

Bodies of aluminum and aluminium alloys were immersed in baths containing solutions having the compositions listed in the second column in Table 1 below and connected as the cathode in a circuit in which an electric current was passed at a voltage and a current density indicated, respectively, in the third and fourth columns of Table 1, for a duration of time indicated in the column headed "T cathode" of the Table. The polarity was then reversed, while the body was kept immersed in the same bath and a current was made to flow at the same voltage and current density for the time specified in the column headed "T anode" of Table 1. The temperatures of the baths employed are listed in the last column of Table 1. In all Examples "H<sub>3</sub>PO<sub>4</sub>" means an aqueous solution containing 85% by weight of pure H<sub>3</sub>PO<sub>4</sub>, and "H<sub>2</sub>SO<sub>4</sub>" means a 66° Bé. aqueous solution. Indications of percentage are all percent v./v., and the current density is measured on the object that is polished.

The same solutions may also be used for polishing aluminium, aluminum alloys and stainless steel.

In all the foregoing Examples 1 to 11, the metal remained during both stages in the same electrolyte. However, the electrolytes may also be changed in the second stage. For example, an aluminium alloy immersed in the first stage in a bath of composition 1 in Table 1 may in the second stage be immersed in any of the other baths indicated in the same Table. The same applies to stainless steel—Table 2, and to copper and its alloys—Table 3.

I claim:

1. A process for the electrolytic polishing of a body made of a metal selected from the group consisting of aluminum, aluminum alloys, copper, copper alloys and stainless steels, comprising

subjecting said body in a first stage for at least one minute to an electrolytic cathodic treatment in an acidic electrolyte containing phosphoric acid and a copper salt in an amount not exceeding 10 g./l. thereby effecting intergranular corrosion in the surface region of said body, and

in a subsequent, second stage, subjecting said body to electrolytic anodic treatment in an acidic electrolyte containing phosphoric acid and no more than 10 g./l. of a copper salt for at least one minute thereby imparting to the body a desired degree of polish, the following conditions being maintained throughout

TABLE 1

| Ex. No. | Composition of the electrolytic bath                                                                                                                                                                  | Voltage in volts | Current density, amp/dm. <sup>2</sup> | T cathode, minutes | T anode, minutes | Temperature, °C. |
|---------|-------------------------------------------------------------------------------------------------------------------------------------------------------------------------------------------------------|------------------|---------------------------------------|--------------------|------------------|------------------|
| 1       | H <sub>3</sub> PO <sub>4</sub> , 55% plus H <sub>2</sub> SO <sub>4</sub> , 45% to which mixture is added: CrO <sub>3</sub> , 7.5 g./l.; CuSO <sub>4</sub> , 3 g./l.; H <sub>2</sub> O dist. 55 cc./l. | 14               | 30                                    | 3                  | 5                | 80               |
| 2       | H <sub>3</sub> PO <sub>4</sub> , 60%; glycerine 40%; CuSO <sub>4</sub> , 5 g./l.                                                                                                                      | 15               | 30                                    | 2                  | 6                | 60               |
| 3       | H <sub>3</sub> PO <sub>4</sub> , 75% H <sub>2</sub> SO <sub>4</sub> , 25% to which mixture is added: HNO <sub>3</sub> , 50 g./l.; CuSO <sub>4</sub> , 5 g./l.                                         | 14               | 10                                    | 2                  | 5                | 85               |

In all cases a highly polished surface was obtained. The same solutions as above may also be used for polishing copper, copper alloys and stainless steel.

said first and second stages:

Voltage \_\_\_\_\_ volts 5-150  
Current density on the body \_\_\_\_ amp/dm.<sup>2</sup> 1-150  
Electrolytic bath temperature \_\_\_\_\_ °C. 20-95

Bodies of stainless steel SS 304 18/8 were submitted to a procedure analogous to that described in Examples 75 electrolyte is used in both stages.

2. A process according to Claim 1, wherein the same

3. A process according to Claim 1, wherein at least during the second stage part of the body surface is covered by an insulating material so that only the non-covered portions of the surface are polished, and the insulating cover is removed after the completion of the second stage.

4. A process according to Claim 1, wherein the body is electrically connected prior to its immersion in the electrolytic solution.

5. A process according to Claim 1, wherein the electrolyte is an aqueous solution of phosphoric acid, sulfuric acid, chromic acid and 1-10 g./l. of a copper salt.

6. A process according to Claim 1, wherein the electrolyte is an aqueous solution containing phosphoric acid, nitric acid, sulfuric acid and 1-10 g./l. of a copper salt.

7. A process according to Claim 1, wherein the electrolyte is an aqueous solution containing phosphoric acid, at least one alcohol and 1-10 g./l. of a copper salt.

8. A process according to Claim 7, wherein the alcohol is propyl alcohol, butyl alcohol or glycerine.

9. A process according to Claim 1, wherein the electrolyte is an aqueous phosphoric acid solution containing 1-10 g./l. of a copper salt.

10. A process according to Claim 1, wherein said copper salt is copper sulfate.

References Cited

UNITED STATES PATENTS

|           |         |           |       |            |
|-----------|---------|-----------|-------|------------|
| 3,287,238 | 11/1966 | Latawiec  | ----- | 204—129.35 |
| 3,519,779 | 7/1970  | Dolomont  | ----- | 204—129.9  |
| 3,389,065 | 6/1968  | Shibasaki | ----- | 204—129.8  |
| 2,366,714 | 1/1945  | Faust     | ----- | 204—129.9  |
| 2,706,171 | 4/1955  | Goral     | ----- | 204—129.9  |

15 THOMAS M. TUFARIELLO, Primary Examiner

U.S. CL. X.R.

204—129